

## UNITED STATES PATENT OFFICE

1,931,266

## PROCESS OF TREATING ARTIFICIAL THREADS

Harold Henry Parker, Kenmore, N. Y., assignor to Du Pont Rayon Company, New York, N. Y., a corporation of Delaware

No Drawing. Application January 10, 1930  
Serial No. 420,019

6 Claims. (Cl. 18—54)

This invention relates to a process of treating artificial threads and more particularly to a process of desulphuring threads produced by the viscose process.

5 In the manufacture of artificial threads by the viscose process, certain sulphur bodies are formed in the coagulation and regeneration steps. These sulphur bodies become associated with the threads and must be removed to make the product salable. In the art, the process of removing the sulphur is known as desulphuring.

The stage in the manufacture of the yarn at which the desulphuring step is employed depends on the process of spinning and the after treatment which is employed. In some processes, the freshly coagulated threads received on a bobbin or in a bucket are wound into skeins and the latter treated for the removal of the adherent liquors and the sulphur. In other processes, 15 after the freshly spun threads collected on a bobbin or in a bucket are washed to remove the acid and other coagulating bath liquors, they are either processed in the form of cakes or bobbins or converted, after drying, into skeins for further treatment, including bleaching and desulphuring. To eliminate the objections inherent in the handling of the freshly spun threads, it is desirable to perform the operations on the threads wound on bobbins, in buckets, or on cakes provided with 20 inserts. It is obvious that the carriers on which the silk is subjected to the treatment must be made of a material resistant to the desulphuring agents employed as well as the bath liquors. Up to the present time the most satisfactory material used for this purpose is aluminum.

The sulphides, particularly the alkali sulphides including sodium sulphide, are the most efficient for removing the sulphur impurities. Their use has, nevertheless, up to this time been seriously limited by the corrosion of the aluminum carriers or other parts of the equipment, which tends to contaminate the threads and results in an inferior product. Thus, prior to this invention, it has been necessary to resort to desulphuring processes which do not utilize the alkali sulphides and are inferior to the alkali sulphide desulphuring operation in economy as well as resulting in a product of poorer quality.

I have found that I can desulphur artificial threads produced from viscose and disposed on aluminum carriers with solutions containing a salt of a weak acid having an alkaline reaction such as an alkali sulphide, said salt normally corroding aluminum, and inhibit the corrosion of the aluminum and contamination of the threads

resulting therefrom by adding to said solution a compound, such as sodium silicate.

It is therefore an object of this invention to provide a method of desulphuring viscose artificial threads on aluminum carriers with a salt of a weak acid having an alkaline reaction and in which method the aluminum carriers are not substantially corroded.

Another object of this invention is to desulphur artificial yarn produced from viscose and disposed on aluminum carriers with a desulphuring composition comprising an alkali sulphide, such as sodium sulphide, and an agent which substantially inhibits the corrosion of the aluminum by the said alkali sulphide.

Another object of this invention is to provide a method of desulphuring artificial yarn produced from viscose and disposed on aluminum carriers which comprises subjecting said yarn and carriers to a desulphuring solution comprising sodium sulphide and sodium silicate.

Other objects will appear from the following description and appended claims.

According to one manner of practicing this invention, freshly spun cakes of artificial threads produced from viscose are removed from the spinning bucket and provided with resilient foraminous aluminum inserts and then placed on washing racks. Water or another solution adapted to remove the coagulating bath liquor from the cakes is allowed to drip onto the cakes for a sufficient time to substantially free them of acid and salts. As hereafter explained, the cakes are then treated with the desulphuring solution whereby the sulphur impurities are removed.

The desulphuring solution which is utilized and which constitutes a part of this invention comprises a salt of a weak acid having an alkaline reaction such as alkali sulphide and which normally corrodes aluminum, and a compound, such as sodium silicate, which inhibits the corrosion of the aluminum by said salts. Various proportions of the ingredients may be employed. Satisfactory results have been obtained with a solution of sodium sulphide containing approximately 0.2% of sodium sulphide and sufficient 40° Bé. water glass to produce 0.1% of silica ( $\text{SiO}_2$ ) in the final solution.

In employing this solution, it is heated to approximately 90° C. and allowed to drip onto the washed cakes of artificial threads until the sulphur is substantially removed from the cakes. The cakes are then given a final wash with water to remove the desulphuring solution, after which

they may be bleached, dyed, sized, or the like before drying.

Hard or soft water may be employed and the treatment may be carried out at any temperature. 5 The best results are attained when the temperature is as near to the boiling point of the solution as practical. Good results, however, are obtained at lower temperatures. For example, I have found that by immersing the cakes in the 10 sodium-sulphide-sodium-silicate solution at 45° C., excellent desulphuring is obtained, particularly if the cakes have previously been dried in order to impart to the cakes of rayon on the insert a somewhat more open texture. A commercially operative and practical process is also obtained when the desulphuring step is carried out at room temperature.

In place of the sodium-sulphide-sodium-silicate solution, a solution containing sodium carbonate and sodium silicate may also be used with success. For this solution, a combination of ingredients is preferred that will produce a combined alkalinity of 0.3% calculated as sodium carbonate and a silica content of 0.05%.

25 If desired, sodium cyanide may be added to the desulphuring solution. The cyanide serves the special purpose of removing from the yarn any traces of the iron and copper resulting from the contamination with parts of the equipment.

30 It is clear that while sodium silicate 40° Bé. water glass is referred to, any other grade of sodium silicate may be used as well, it being necessary to make only such adjustment of the alkalinity of the solution so that the silica will not precipitate.

35 Though the invention has been described with particular reference to desulphuring of cakes, it is applicable to the desulphuring of threads wound on bobbins, skeins, or in spinning buckets. 40 It is equally applicable to yarn which has been dried or to threads in the gel state, that is, those threads which have not been submitted to any drying operation. The desulphuring process may be also successfully practiced by immersing the 45 yarn in the solution, by pressure or vacuum desulphuring, or by centrifugal desulphuring.

50 Since it is obvious that various changes and modifications may be made in the specific details above described, this invention is not restricted thereto except as set forth in the appended claims.

I claim:

1. The process of desulphuring threads pro-

duced from viscose and disposed on aluminum carriers which comprises subjecting said threads and carriers to a solution containing a salt of a weak acid having an alkaline reaction and which normally corrodes aluminum and sodium silicate, said silicate inhibiting the corrosion of said carriers by said salt, said solution having an alkalinity content of 0.3% calculated as sodium carbonate and a silica content of 0.05% to 1%.

80 2. The process of desulphuring threads produced from viscose and disposed on aluminum carriers which comprises subjecting said threads and carriers to a solution containing 0.2% of sodium sulphide and sodium silicate in an amount sufficient to produce a silica content of 0.10%.

85 3. The process of desulphuring threads produced from viscose and disposed on aluminum carriers which comprises subjecting said threads and carriers to a solution containing sodium carbonate and sodium silicate in such proportions that the combined alkalinity will be 0.3% calculated as sodium carbonate and the silica content 0.05%.

90 4. A process which comprises subjecting threads produced from viscose and disposed on aluminum carriers to a desulphuring solution containing a salt of a weak acid having an alkaline reaction and which normally corrodes aluminum as the effective desulphuring agent 100 and a sufficient quantity of sodium silicate to inhibit the corrosion of said carriers by the desulphuring agent, the total alkalinity of the desulphuring solution being such as will prevent the precipitation of silica.

95 5. A process which comprises subjecting threads produced from viscose and disposed on aluminum carriers to a desulphuring solution containing an alkali sulphide and a sufficient quantity of sodium silicate to inhibit the 110 corrosion of said carriers by said alkali sulphide, the total alkalinity of said solution being such as to prevent the precipitation of silica.

115 6. A process which comprises subjecting threads produced from viscose and disposed on aluminum carriers to a desulphuring solution containing an alkali carbonate and a sufficient quantity of sodium silicate to inhibit the 120 corrosion of said carriers by said alkali carbonate, the total alkalinity of said solution being such 125 as to prevent the precipitation of silica.

HAROLD HENRY PARKER.

55

130

60

135

65

140

70

145

75

150